



US006458244B1

(12) **United States Patent**  
Wang et al.

(10) **Patent No.:** US 6,458,244 B1  
(45) **Date of Patent:** Oct. 1, 2002

(54) **SYNTHETIC FIBER PAPER**(75) Inventors: **Xingli Wang; Shiyi Tao**, both of Chengdu (CN)(73) Assignee: **Sichuan Foreign Economic Relations & Trade Corporation**, Chengdu (CN)

( \*) Notice: Subject to any disclaimer, the term of this patent is extended or adjusted under 35 U.S.C. 154(b) by 0 days.

(21) Appl. No.: **09/488,333**(22) Filed: **Jan. 20, 2000**(30) **Foreign Application Priority Data**

Jan. 22, 1999 (CN) ..... 99114635 A

(51) **Int. Cl.<sup>7</sup>** ..... **D21H 13/24; D21H 13/26; D21H 17/68; D21H 27/12**(52) **U.S. Cl.** ..... **162/146; 162/138; 162/149; 162/157.3; 162/181.6; 442/415; 442/169; 428/324; 428/338**(58) **Field of Search** ..... 162/158, 148, 162/146, 145, 149, 138, 157.3, 168.1, 181.1, 181.6, 181.7; 428/326, 323, 338, 324, 327; 442/415, 93, 117, 147, 168-169(56) **References Cited**

## U.S. PATENT DOCUMENTS

|             |   |         |             |       |           |
|-------------|---|---------|-------------|-------|-----------|
| 3,168,434 A | * | 2/1965  | Heyman      | ..... | 162/146   |
| 3,622,445 A | * | 11/1971 | Heidweiller | ..... | 162/145   |
| 3,756,908 A | * | 9/1973  | Gross       | ..... | 162/146   |
| 4,320,081 A | * | 3/1982  | Lammers     | ..... | 264/184   |
| 4,541,894 A | * | 9/1985  | Cassat      | ..... | 162/138   |
| 4,698,267 A | * | 10/1987 | Tokarsky    | ..... | 428/474.4 |

|              |   |         |                  |       |         |
|--------------|---|---------|------------------|-------|---------|
| 4,714,650 A  | * | 12/1987 | Obayashi et al.  | ..... | 442/93  |
| 4,729,921 A  | * | 3/1988  | Tokarsky         | ..... | 428/326 |
| 5,336,556 A  | * | 8/1994  | Yoshida et al.   | ..... | 442/414 |
| 5,403,444 A  | * | 4/1995  | Goettmann et al. | ..... | 162/146 |
| 5,415,738 A  | * | 5/1995  | Methta et al.    | ..... | 162/146 |
| 5,783,039 A  | * | 7/1998  | Murayama         | ..... | 162/146 |
| 6,171,443 B1 | * | 1/2001  | Goettmann et al. | ..... | 162/135 |

## FOREIGN PATENT DOCUMENTS

|    |              |        |         |
|----|--------------|--------|---------|
| EP | 0 156 587    | 3/1985 |         |
| EP | 0 344 318 A1 | *      | 12/1989 |
| EP | 0 391 6465   | 4/1990 |         |
| EP | 0 681 620 B1 | *      | 11/1995 |
| EP | 0 854 213 A1 | *      | 7/1998  |
| EP | 0 289 860 A1 | *      | 11/1998 |

\* cited by examiner

Primary Examiner—Jose Fortuna

(74) Attorney, Agent, or Firm—Cohen, Pontani, Lieberman &amp; Pavane

(57) **ABSTRACT**

The present invention provides a synthetic fiber paper, the synthetic fiber paper comprises poly (phenylene terephthal amide) fiber, polyethylene glycol terephthalate fiber and powdered mica. The synthetic fiber paper has high-temperature resistance, high strength, low-deformability, resistivity against fire, burning resistance, resistance to chemical corrosion and excellent property of electric insulation, it can be widely applied in the field of mechano-electronics product, aviation, aerospace, military project for national defence, high-tech areas for civil use, high-voltage equipment, high-temperature circumstance as insulting material, it often can be used in composite materials with special use as structural material. The present invention also provides a process for preparing this synthetic fiber paper.

**8 Claims, 1 Drawing Sheet**



FIG. 1

## SYNTHETIC FIBER PAPER

## FIELD OF THE INVENTION

This invention relates to a synthetic fiber paper, particularly to a fiber paper made of aromatic polyamide synthetic fiber as main raw material; this invention also relates to a process for preparing the synthetic fiber paper.

## DESCRIPTION OF THE PRIOR ART

The synthetic fiber paper of aromatic polyamide is a paper-like material made of synthetic fiber of aromatic polyamide as raw material through a special papermaking technology. Owing to high-temperature resistance, high strength, low-deformability, resistivity against fire, burning resistance, resistance to chemical corrosion and excellent property of insulation, it has been widely used in some high-tech areas such as mechano-electronics product, aviation, aerospace etc. At present, the fiber paper of aromatic polyamide sold on the market, trade name being called as "Nomex Brand paper", uses the fiber of poly (m-phenylene metaphthal amide). However, there is no any satisfied process for preparing the said synthetic fiber paper has been disclosed yet.

## SUMMARY OF THE INVENTION

In view of the shortage of the prior art, the object of the present invention is to provide a synthetic fiber paper made of poly (p-phenylene terephthal amide) as raw material. This fiber paper has high-temperature resistance, high strength, low-deformability, resistivity against fire, burning resistance, resistance to chemical corrosion and excellent property of insulation.

The another object of the present invention is to provide a process for preparing a synthetic fiber paper made of poly (p-phenylene terephthal amide) fiber as raw material.

The present invention provides a synthetic fiber paper comprises (parts by weight):

|                                           |       |
|-------------------------------------------|-------|
| Poly (p-phenylene terephthal amide) fiber | 50-80 |
| Polyethylene glycol terephthalate fiber   | 20-50 |
| Powdered mica                             | 0-50  |

Preferably, the above-mentioned synthetic fiber paper comprises (parts by weight):

|                                           |       |
|-------------------------------------------|-------|
| Poly (p-phenylene terephthal amide) fiber | 70-80 |
| Polyethylene glycol terephthalate fiber   | 20-30 |

The no-stuffing synthetic fiber paper can be produced in proportion as aforesaid content.

More preferably, the above-mentioned synthetic fiber paper comprises (parts by weight):

|                                           |       |
|-------------------------------------------|-------|
| Poly (p-phenylene terephthal amide) fiber | 60-70 |
| Polyethylene glycol terephthalate fiber   | 30-40 |
| Powdered mica                             | 0-10  |

The low stuffing synthetic fiber paper can be produced in proportion as aforesaid content. Powdered mica with 5-20  $\mu\text{m}$  is preferably used in present invention.

More preferably, the above-mentioned synthetic fiber paper comprises (parts by weight):

|                                           |       |
|-------------------------------------------|-------|
| Poly (p-phenylene terephthal amide) fiber | 50-60 |
| Polyethylene glycol terephthalate fiber   | 40-50 |
| Powdered mica                             | 10-15 |

10 The high stuffing synthetic fiber paper can be produced in proportion as aforesaid content.

The said poly (p-phenylene terephthal amide) fiber is 1.5-2.0—, in size, 4-6 m/m in length. The polyethylene glycol terephthalate fiber is 1.5-2.0—in size and 4-6 m/m in length.

15 The process for preparing the synthetic fiber paper comprising the following steps of compounding and pulping, papermaking shaping, dehydrating, drying preheating, prepressing, high-pressure hot-rolling, trimming, wherein the untreated poly (p-phenylene terephthal amide) fiber and the polyethylene glycol terephthalate fiber are in proportion loosened and dissociated before the step of compounding and pulping, then mixing with the treated poly (p-phenylene terephthal amide) fiber to compound and pulp.

20 25 The proportion between the said untreated poly (p-phenylene terephthal amide) fiber and the treated poly (p-phenylene terephthal amide) fiber is preferably 1:1-0.2 by weight, more preferably is 1:0.34 by weight.

In the said process, before compounding and pulping, the 30 powdered mica should be also mixed with the processing additives to be a homogeneous material.

The said processing additives are an inorganic gel and/or polyethylene glycol oxide.

35 In the process of present invention, the preheating temperature is 240-250° C., the prepressing pressure is 1-2 Mpa, the temperature of high-pressure hot rolling is 255-265° C. and the linear pressure is 500-3000 N/cm.

## DETAILED DESCRIPTION OF THE INVENTION

40 The poly (p-phenylene terephthal amide) fiber (Aromatic polyamide fiber 1414) is a structure fiber with general formula as follow:



45 It can be produced by a process comprising following steps: terephthaloyl chloride and p-phenylene diamine as raw material, are polycondensed in NMP—CaCl<sub>2</sub> as solvent under low-temperature to poly (p-phenylene terephthal amide) resin, then undergoing liquid crystal spinning, being cut to length as required, or is precipitated directly to short fiber. The fiber has outstanding high strength (the highest tensile strength 200 CN/betx, shearing 0.29, elongation at rupture 3%), high modulus of elasticity (up to 67 KN/mm<sup>2</sup>), high hot resistance (decomposition point 500° C.), resistivity against fire, burning resistance, resistance to chemical corrosion and excellent property of insulation, therefore the synthetic fiber paper made of poly (p-phenylene terephthal amide) as a main component of structural fiber also has the above-mentioned outstanding excellent properties.

50 55 60 Because of insufficient binding force of the synthetic fibers, the synthetic fibers can not be papermaking shaping

as a plant fiber does. Binding of the synthetic fibers depends mainly on adhesion of melted fiber. However the poly (p-phenylene terephthal amide) fiber doesn't have a distinct melting point, therefore during papermaking shaping some fiber having lower melting point present as crosslinking fiber has to be added. When the paper blank of synthetic fiber is rolled at nearly melting point of the crosslinking fiber, the soft and melted crosslinking fiber binds the unmelted poly (p-phenylene terephthal amide) fiber to form net-like material, so as to be finalized. In this invention the polyethylene glycol terephthalate fiber (polyester fiber) is used as the crosslinking fiber. Its structural formula:



The softening point of the fiber is 238–240° C., melting point is 255–260° C. The fiber has higher softening temperature than using temperature of the synthetic fiber paper 220° C., and higher strength, excellent electric insulation. That the polyethylene glycol terephthalate fiber is added properly as a crosslinking fiber doesn't drop the physical mechanical index and electric insulation of the synthetic fiber paper too much. While stuffing is used, the amount of the crosslinking fiber used in the present invention preferably increases to 40–50 parts by weight, most preferably increases to 30 parts by weight.

When the synthetic fiber paper is used in place where there are high-voltage and frequent or uninterrupted corona discharge being used, it is necessary to add and mix the powdered mica while papermaking, the ability for products resisting to corona discharge is strengthened by stuffing of powdered mica. The proportion of stuffing level depends on its uses, varying from 0 to 50 parts by weight. While the stuffing level reaches 50 parts by weight (high stuffing), the product also has the properties of mica besides the properties of original high strength and high-temperature resistance etc.

In the process for preparing the synthetic fiber paper of the present invention, in order to increase dispersion of fiber in water, while mixing and pulping, a micro-level of high viscosity material should be added to get the pulp slurry to have some viscosity, increases the movement resistance of fiber in the pulp, delays the twining and flocculating of fiber, so as to improve dispersing and suspending of the fiber in pulp, finally achieves the aim of increasing homogeneity of the synthetic fiber paper.

The micro-level of residual viscosity increaser in the paper blank for papermaking shaping makes the fiber some adhesion, so that it makes the paper blank retain initial strength before finalizing, and will not get rupture in the process of transporting pulling apart from a foundation fabric. The process of papermaking can run smoothly.

The viscosity increaser used in this invention can be selected from a group consisting of inorganic gel SM and polyethylene glycol Oxide PO. They can be either used separately, or as combination. The amount of it is about 0.3–0.8%. It can be able to be adjusted, depending on the viscosity of viscosity increaser, the type, gauge of paper and the type of papermaking machine. In general, the use level for thick paper is adequately more than for thin. The use level for stuffing paper is more than for no—stuffing.

In order to improve the homogeneity of paper blank for papermaking, it is very necessary for the poly (p-phenylene terephthal amide) fiber to have surface-preparation. This

surface-preparation changes the properties of fiber surface, enhances an affinity of fiber to water, so that the dispersing and suspending fiber in water persists for a longer time. There are many process for treating poly (p-phenylene terephthal amide) fiber. Here is a mechanical process or a mechano-chemical combined process is used. It means that the poly (p-phenylene terephthal amide) fiber is beaten by a beater, then it will be shorn and torn to reduce the length of fiber and to make its surface roughness. While beating, the micro-level of processing additives also can be added, after that it will be mixed and beaten, it is what is called the mechano-chemical combined process. In practical production, it is also possible to apply poly (p-phenylene terephthal amide) fibers in two different lengths combined (especially suitable for super short fiber which is directly produced by precipitating process). Same effect result can be achieved.

Because the synthetic fiber paper should have both a better tensile strength, elongation rate, density, and a higher tearing strength, initial tear, at the same time, it also should have the property of the best homogeneity in the process of papermaking, in order to resolve the contradiction between demanding fiber length of the tearing strength and of tensile strength, in present invention, a certain amount of untreated poly (p-phenylene terephthal amide) (long fiber) as skeleton of paper blank compounded in part of treated poly (p-phenylene terephthal amide) fiber(short fiber) is compounded in part and stuffed in the skeleton of the poly (p-phenylene terephthal amide) fiber to be untreated, the interweaving of long fiber with short fiber trends further towards homogeneity, thereby enhances the papermaking homogeneity of the paper blank and the interweaving density of fibers.

TABLE 1

| The effects on physical, mechanical properties of paper blank by compounding proportion of two types of poly (p-phenylene terephthal amide) fibers |                                    |                                                |                                                     |                                                |                                         |
|----------------------------------------------------------------------------------------------------------------------------------------------------|------------------------------------|------------------------------------------------|-----------------------------------------------------|------------------------------------------------|-----------------------------------------|
|                                                                                                                                                    | Untreated fibers<br>Treated fibers | Density of<br>paper blank<br>g/cm <sup>3</sup> | Tearing strength<br>index<br>CN • m <sup>2</sup> /g | Initial<br>tear index<br>N • m <sup>2</sup> /g | Tensile<br>strength<br>index<br>N • m/g |
| 40                                                                                                                                                 | 1:1                                | 0.19                                           | 2.48                                                | 0.44                                           | 27.7                                    |
|                                                                                                                                                    | 1:0.34                             | 0.20                                           | 3.75                                                | 0.61                                           | 20.7                                    |
| 45                                                                                                                                                 | 1:0.2                              | 0.21                                           | 5.21                                                | 0.73                                           | 9.24                                    |

It can be noted from table 1 that the tearing strength and initial tear increase as the use level of treated fibers increases, the tensile strength reduces as the use level of untreated fibers increases. The ratio of two types of poly (p-phenylene terephthal amide) fibers is preferably adjusted to 1:0.34 thereby all relative properties are kept with satisfaction. When there are some special demands for the tearing strength and the tensile strength of paper due to different use, a satisfied products still can be produced through adjusting the ratio of two kinds of poly (p-phenylene terephthal amide) fibers based on the indication shown in table 1.

After the synthetic fiber paper is dried, because of weak adhesives force between fibers, the fiber of paper blank is slack, its mechanical properties are weak, accordingly, it has to be given treated by the hot-rolling setting to make the crosslink fiber (short cut filament of polyester) with low melt point soften, melt, and under the pressure it will be made to bind with the fiber net made of untreated poly (p-phenylene terephthal amide) fiber and to be finalized, thereby it will be made to have required properties.

In order to make the paper blank have sufficient mechanical strength to bear the strong tensile and prevent it from being rupture when hot-rolling at high pressure, before the step of hot-rolling at high pressure, the paper blank should be passed through the preheating roller to preheat it to the softening point of crosslinking fiber, and a lower prepressing pressure should be exerted on to make paper blank has sufficient mechanical strength.

TABLE 2

| Hot-rolling temperature and pressure |                              |                                   |                                                  |
|--------------------------------------|------------------------------|-----------------------------------|--------------------------------------------------|
| Preheating prepressing               | Hot-rolling at high pressure |                                   |                                                  |
| preheating temperature (° C.)        | prepressing pressure (Mpa)   | temperature of hot-rolling (° C.) | linear pressure of hot-rolling N/cm <sup>2</sup> |
| 240~250                              | 1~2                          | 255~265                           | 500~3000                                         |

The higher the hot-rolling pressure is, the greater the density of the synthetic fiber paper will be. By means of changing the pressure of roller (linear pressure), a various types of products with different density can be obtained.

When stuffing is being filled, in order to make the stuffing attain has enough adhesion, more crosslinking fiber should be made to be melted, at the same time the hot-rolling temperature should be properly to 265° C.

The process can be operated smoothly by mixing the stuffing (powered mica) with micro-level of processing additives while stirred at high speed to form pulp, then the result mixture was compounded into the pulp of fiber paper.

In order to prevent the crosslinking fiber from being over melted and the technical properties of synthetic fiber paper being affected. The temperature of preheating and hot-rolling should be controlled precisely at a point of temperature selected, the error in temperature is ±1° C.

Because the heat conductivity coefficient of paper blank is lower, its heat conduction is slow, the thicker the synthetic fiber paper is, the longer the preheating time will be.

The synthetic fiber paper of the present invention is a kind of new synthetic material with high performance. It is a paper-like material made of the synthetic fiber of aromatic polyamide as main component and produced by special papermaking technology. It has high-temperature resistance (suitable used to be at -190~310° C., and can be used for long time below 220° C.), high strength, low-deformability, resistivity against fire, burning resistance, resistivity to chemical corrosion and excellent property of electric insulation. The low-density, middle-density, high-density paper of synthetic fiber can be produced by the means of changing the character of fiber, the ratio of two fibers, hot-rolling pressure as required according to the different use.

The type of no-stuffing, low-stuffing and high-stuffing products can be produced by means of changing the proportion of stuff to be added. The products also can be made to have different thickness gauge (0.05~10 mm) (if more than 1.0 mm, be called as fiber paperboard) and different width gauge. The present invention can provide a series of products with different type and different gauge to meet the needs in different technical areas. The synthetic fiber paper in the present invention can be widely applied in the field of mechano-electronics, aviation, aerospace, military project for national defense, high-tech areas for civil use, high-voltage equipment, high-temperature circumstance as insulating material, besides, it often can be used in composite material with special use as structural material.

## BRIEF DESCRIPTION OF DRAWINGS

FIG. 1 is a flow diagram process for preparation of the present invention.

## EXAMPLES

## Example 1

According to following proportion, the synthetic fiber paper of example 1 was produced by a process of the present invention.

|                                           |       |
|-------------------------------------------|-------|
| Poly (p-phenylene terephthal amide) fiber | 70 kg |
| Polyethylene glycol terephthalate fiber   | 30 kg |

The above-mentioned poly p-phenylene terephthal amide fiber comprises 52 kg of untreated poly (p-phenylene terephthal amide) fiber having -1.5 d—in size and 6 m/m in length and 18 kg of the treated poly (p-phenylene terephthal amide) fiber. The polyethylene glycol terephthalate fiber is -1.5 d—in size and 6 m/m in length.

The above-mentioned process of the present invention comprises:

Referring to FIG. 1, the untreated poly (p-phenylene terephthal amide) fiber were subjected to be loosened and dissociated, then was compounded with the treated poly (p-phenylene terephthal amide) fiber to make pulp, through the steps of papermaking shaping, dehydrating, drying, preheating and prepressing at 245° C. and under 2 Mpa, hot-rolling under 600 N/cm of linear pressure and at 260° C., so as to make a no-stuffing synthetic fiber paper with low density of 0.3~0.5 g/cm<sup>3</sup>; then trimming, rolling-up, to obtain the product. The wastewater from dehydrating can be recycled after it was treated as required.

## Example 2

According to the process indicated as example 1, except that the hot-rolling pressure during the stage of high pressure hot-rolling was 1200 N/cm. Finally a no-stuffing middle-density synthetic fiber paper having density of 0.5~0.99 g/m<sup>3</sup> was obtained.

## Example 3

The same ratio of two synthetic fiber papers and process as described for example 1 were used except that the linear pressure at high-pressure hot-rolling is 3000 N/cm. Finally no-stuffing high-density synthetic fiber paper having density of 0.9~1.2 g/cm<sup>3</sup> was obtained.

## Example 4

According to following proportion, the synthetic fiber paper of example 4 was produced by a process substantially same as the process described in example 1:

|                                           |       |
|-------------------------------------------|-------|
| Poly (p-phenylene terephthal amide) fiber | 65 kg |
| Polyethylene glycol terephthalate fiber   | 30 kg |
| Powdered mica (5~10 μm in graininess)     | 1 kg  |

The above-mentioned poly (p-phenylene terephthal amide) fiber comprises 45 kg of untreated poly (p-phenylene terephthal amide) fiber with -1.5 d—in size and 6 m/m in length and 20 kg of treated poly (p-phenyl terephthal amide)

fiber. The polyethylene glycol terephthalate fiber with -1.5 d—in size and 4 m/m in length is adapted.

The process of example 4 is substantially same as the process described in example 1, except that before compounding and pulping, powdered mica, water and micro-level of processing additives—polyethylene glycol oxide have to be mixed and homogenized, then they are added to the above-mentioned composition consisting of poly (p-phenylene terephthal amide) fiber and polyethylene glycol terephthalate fiber to be made compound and pulp; preheating temperature is 250° C., prepressing pressure is 1.5 Mpa; the temperature at the high-pressure hot-rolling is 265° C., the linear pressure is 1500 N/cm.

#### Example 5

According to following proportion, compound and manufacture the synthetic fiber paper in example 5 was produced

|                                            |       |
|--------------------------------------------|-------|
| Poly (p-phenylene terephthal amide) fiber  | 50 kg |
| Polyethylene glycol terephthalate fiber    | 50 kg |
| Powdered mica (5–10 $\mu$ m in graininess) | 50 kg |

The above-mentioned poly (p-phenylene terephthal amide) fiber comprises 40 kg of untreated poly (p-phenylene terephthal amide) fiber having -1.5 d—in size and 6 m/m in length and 10 kg of treated poly (p-phenylene terephthal amide) fiber. The polyethylene glycol terephthalate fiber adopted is -2.0d—in size and 6 m/m in length.

The process used in example 5 is same as the process described in example 4.

#### Example 6

According to the following proportion, compound and manufacture the synthetic fiber paper of example 6 was produced:

|                                             |       |
|---------------------------------------------|-------|
| Poly (p-phenylene terephthal amide) fiber   | 60 kg |
| Polyethylene glycol terephthalate fiber     | 40 kg |
| Powdered mica (10–15 $\mu$ m in graininess) | 10 kg |

The above-mentioned poly (p-phenylene terephthal amide) fiber comprises 45 kg of the untreated poly (p-phenylene terephthal amide) fiber having 2 D in size and 6 m/m in length and 15 kg of the treated poly (p-phenylene terephthal amide) fiber. The polyethylene glycol terephthalate fiber used is 2 D in size and 6 m/m in length.

The process of example 6 is substantially same as the process described in example 4, except that the high-pressure hot-rolling was carried out at 265° C. and 2000 N/cm of the linear pressure.

#### Example 7

According to following proportion, compound and manufacture the synthetic fiber paper of example 7 was produced:

|                                             |       |
|---------------------------------------------|-------|
| Poly (p-phenylene terephthal amide) fiber   | 60 kg |
| Polyethylene glycol terephthalate fiber     | 40 kg |
| Powdered mica (10–20 $\mu$ m in graininess) | 10 kg |

The above-mentioned poly (p-phenylene terephthal amide) fiber comprises 40 kg of the untreated poly

(p-phenylene terephthal amide) fiber having -1.5 d—in size and 6 m/m in length and 20 kg of the treated poly (p-phenylene terephthal amide) fiber. The polyethylene glycol terephthalate fiber adopted is -1.5 d—in size and 4 m/m in length.

The production process of example 7 is substantially same as the process described in example 6.

#### Example 8

According to following proportion, compound and manufacture the synthetic fiber paper of example 8 was produced:

|                                             |       |
|---------------------------------------------|-------|
| Poly (p-phenylene terephthal amide) fiber   | 50 kg |
| Polyethylene glycol terephthalate fiber     | 50 kg |
| Powdered mica (10–20 $\mu$ m in graininess) | 50 kg |

The above-mentioned poly (p-phenylene terephthal amide) fiber comprises 30 kg of the untreated poly (p-phenylene terephthal amide) fiber having -1.5 d—in size and 6 m/m in length and 20 kg of the treated poly (p-phenylene terephthal amide) fiber. The polyethylene glycol terephthalate fiber used was -1.5 d—in size and 5 m/m in length.

The process of example 8 is substantially same as the process described in example 6.

#### Example 9

According to following proportion, compound and manufacture the synthetic fiber paper of the example 9 was produced

|                                           |       |
|-------------------------------------------|-------|
| Poly (p-phenylene terephthal amide) fiber | 50 kg |
| Polyethylene glycol terephthalate fiber   | 50 kg |

The above-mentioned poly (p-phenylene terephthal amide) fiber was -1.5 d—in size and 6 m/m in length. The polyethylene glycol terephthalate fiber was -1.5 d—in size and 4 m/m in length. The process is substantially same as the process described in example 3, except that the beating process was carried out prior to compounding.

Although particular embodiments of the present invention have been described in the foregoing description, it will be understood by those skilled in the art that the invention is capable of numerous modifications, substitutions and rearrangements without departing from the spirit or essential attributes of the invention. Reference should be made specification, as indicating the scope of the invention.

What is claimed is:

1. A synthetic fiber paper comprising:

|                                           |                       |
|-------------------------------------------|-----------------------|
| Poly (p-phenylene terephthal amide) fiber | 50–80 parts by weight |
| Polyethylene glycol terephthalate fiber   | 20–50 parts by weight |
| Powdered mica                             | 0–50 parts by weight  |

wherein said Polyethylene glycol terephthalate fiber has a melting point of about 255–260° C.

2. Synthetic fiber paper according to claim 1, wherein said synthetic fiber paper comprising:

|                                           |                        |
|-------------------------------------------|------------------------|
| Poly (p-phenylene terephthal amide) fiber | 70–80 parts by weight  |
| Polyethylene glycol terephthalate fiber   | 20–30 parts by weight. |

**3.** Synthetic fiber paper according to claim **2**, wherein said poly (p-phenylene terephthal amide) fiber is 1.5–2.0 d—in size and 4–6 m/m in length and said polyethylene glycol terephthalate fiber is 1.5–2.0 d—in size and 4–6 m/m in length.

**4.** Synthetic fiber paper according to claim **1**, wherein said synthetic fiber paper comprising:

|                                           |                       |
|-------------------------------------------|-----------------------|
| Poly (p-phenylene terephthal amide) fiber | 60–70 parts by weight |
| Polyethylene glycol terephthalate fiber   | 30–40 parts by weight |
| Powdered mica                             | 0–10 parts by weight. |

**5.** Synthetic fiber paper according to claim **4**, wherein said poly (p-phenylene terephthal amide) fiber is 1.5–2.0 d—in

size and 4–6 m/m in length and said polyethylene glycol terephthalate fiber is 1.5–2.0 d—in size and 4–6 m/m in length.

**6.** Synthetic fiber paper according to claim **1**, wherein said synthetic fiber paper comprising:

|                                           |                        |
|-------------------------------------------|------------------------|
| Poly (p-phenylene terephthal amide) fiber | 50–60 parts by weight  |
| Polyethylene glycol terephthalate fiber   | 40–50 parts by weight  |
| Powdered mica                             | 10–50 parts by weight. |

**7.** Synthetic fiber paper according to claim **6**, wherein said poly (p-phenylene terephthal amide) fiber is 1.5–2.0 d—in size and 4–6 m/m in length and said polyethylene glycol terephthalate fiber is 1.5–2.0 d—in size and 4–6 m/m in length.

**8.** Synthetic fiber paper according to claim **1**, wherein said poly (p-phenylene terephthal amide) fiber is 1.5–2.0 d—in size and 4–6 m/m in length and said polyethylene glycol terephthalate fiber is 1.5–2.0 d—in size and 4–6 m/m in length.

\* \* \* \* \*